

## UNITED STATES PATENT OFFICE

CONWAY VON GIRSEWALD, OF FRANKFORT-ON-THE-MAIN, GERMANY

## PROCESS FOR THE PRODUCTION OF ALUMINUM-SILICON ALLOYS FREE FROM CARBIDE

No Drawing. Application filed May 8, 1926, Serial No. 107,788, and in Germany May 12, 1925.

This invention relates to a process for the production by electro-thermic means, of aluminum silicon alloys practically free from carbide.

5 It is known to produce aluminum silicon alloys rich in iron by electro-thermic means. Such alloys are employed as deoxidizing agents, the high iron content about 10 to 30% not interfering with their use. However 10 owing to this high iron content, these alloys cannot be employed in the production of pure aluminum silicon alloys capable of being cast.

If however correspondingly pure i. e., almost iron-free initial materials are employed, 15 it is possible to produce by electro-thermic treatment, an aluminum silicon alloy which is almost free of iron. Nevertheless it is impossible to obtain in this manner an alloy which has the composition of commercial,

20 aluminum alloys containing for example 8 or 13% silicon. At the high reduction temperatures of the oxides prevailing in the electric furnace carbon is taken up and such large amounts of carbides are formed that the alloy 25 cannot be industrially employed as a casting alloy. If however the silicon content is increased up to 35% and over, by suitably proportioning the ingredients of the furnace charge, the surprising observation is made, 30 that the formation of carbide disappears practically completely. It should be remarked that even a comparatively small proportion of carbon, is detrimental for the manufacture as well as for the employment 35 of the alloy for casting purposes.

The alloys rich in silicon must be alloyed with pure aluminum in accordance with the purpose for which they are to be used. Nevertheless if the preliminary alloy contains for

40 example 2 to 3% carbon, subsequent alloying is practically impossible. If however the preliminary alloy contains a smaller proportion, for example 1 to 2%, of carbon, then part of the alloy will proceed to alloy, but so 45 much residue remains in the form of carbon containing dross, that the process becomes uneconomical.

The discovery that an alloy of aluminum containing more than 35% silicon hardly 50 takes up any carbon is the more surprising,

as it is well known that both pure aluminum as well as pure silicon, form corresponding carbides with carbon at 1400° C.

The preliminary alloy produced according to the present process can be alloyed with 55 pure aluminum, and thereupon worked up to the known aluminum silicon alloys, the usual known additions being also employed if desired. It is immaterial whether these substances such as for example, small amounts 60 of copper, are added during the formation of the subsequent alloy or are already present in the preliminary alloy produced by electrothermic means.

What I mean by the expression "practically iron-free" in the appended claims is an alloy whose iron content does not exceed 2%, —preferably an alloy containing less than 1% of iron.

I claim:

1. In a process for the production of practically carbide-free aluminum-silicon alloys by electro-thermic means, the step which comprises the production of a practically iron-free preliminary alloy containing upwards 75 of 35% of silicon.

2. In a process for the production of practically carbide-free aluminum-silicon alloys by electro-thermic means the step which comprises the production of a practically iron-free 80 preliminary alloy containing between 35% to 47% silicon.

3. A process for the production of practically carbide-free aluminum-silicon alloys by electro-thermic means, which comprises the 85 production of a practically iron-free preliminary alloy containing upwards of 35% of silicon and alloying said preliminary alloy with pure aluminum.

4. A process for the production of practically carbide-free aluminum-silicon alloys by electro-thermic means, which comprises the production of a practically iron-free preliminary alloy containing upwards of 90 35% of silicon, alloying said preliminary alloy in admixture with other known metals, to aluminum.

5. In a process for the production of practically carbide-free aluminum alloys by electro-thermic means the step which comprises elec- 95 100

trically heating to alloying temperature in the presence of reducing agents practically iron-free aluminum compounds with practically iron-free silicon compounds in such 5 proportions that the resulting practically iron-free aluminum alloys contain not less than 35% of silicon.

6. In a process for the production of practically carbide-free aluminum alloys by electro-thermic means the step which comprises 10 heating to alloying temperature in an electric furnace and in the presence of reducing agents practically iron-free aluminum compounds with practically iron-free silicon 15 compounds in such proportions that the resulting practically iron-free aluminum alloys contain not less than 35% of silicon.

In testimony whereof I affix my signature.  
CONWAY VON GIRSEWALD.

20

25

30

35

40

45

50

55

60

65